

## UNITED STATES PATENT OFFICE

2,338,920

PROCESS FOR THE MANUFACTURE OF  
ARTIFICIAL TEXTILE FIBERSAntonio Ferretti, Milan, Italy; vested in the  
Alien Property CustodianNo Drawing. Application July 31, 1940. Serial  
No. 348,994. In Italy August 28, 1935

4 Claims. (Cl. 18—54)

This invention concerns improvements in or relating to processes for the manufacture of artificial textile fibers.

In co-pending U. S. patent application Serial No. 96,470, of 1936, of which this application is a continuation in part, processes are described and claimed by which a casein and a colloidal solution thereof may be produced which are suitable for use in the manufacture of artificial textile fabrics. The present invention concerns the treatment of such casein when spinning.

According to the present invention there is provided in a process for the manufacture of artificial textile fibers, the step of passing an alkaline solution of casein derived from milk through a spinning nozzle and coagulating the filaments obtained thereby in an aqueous solution of an acid and at least one other substance which renders the coagulated fibers insoluble. The process may be effected with the addition of aluminium salts and/or tin salts and/or formaldehyde with or without sodium salts to the acid coagulating bath.

Example of coagulating baths which may be employed are as follows:

## Example A

An aqueous solution of sulphuric acid and sodium sulphate is made, the proportions being such that the bath contains 140 cubic centimetres of 66° Bé. sulphuric acid and 400 grammes of sodium sulphate for each litre of the bath. To this solution, aluminium salts are added, preferably aluminium sulphate or potash alum. It is also advantageous to add small quantities of tin salts, for example tin acetate.

## Example B

An aqueous solution of sulphuric acid, aluminium sulphate (or potash alum) and sodium chloride is made, the proportions being such that the bath contains, for each litre thereof, 150 cubic centimetres of 66° Bé. sulphuric acid, 150—200 grammes of aluminium sulphate and 75 grammes of sodium chloride. The quantity and proportion of aluminium sulphate and sodium chloride may be varied according to the effects required, bearing in mind that the function of the aluminium salts is to harden rapidly the filaments as soon as they have been coagulated, and that the presence of the sodium chloride in the bath assists the action of the aluminium salts in making filaments insoluble. In preparing this solution, care should be taken not to heat it unduly, so as to avoid the transformation of a portion of the sulphuric acid into hydrochloric acid. There may

likewise be added to this solution small quantities, up to 10% of the solution by weight, of other salts, such as for example, magnesium sulphate, zinc sulphate, ammonium sulphate or the like in order to increase the efficiency of the coagulation.

When the colloidal solution of casein contains carbon disulphide, it is preferable to employ the first bath indicated above as the coagulating agent.

For the mixed solutions of casein and viscose, the first bath is likewise preferable and the amount of sulphuric acid employed can be gradually reduced to 55% of the amount indicated above according to the higher or lower percentage of viscose added to the casein solution. The higher the percentage of viscose, the lower can be the amount of acid in the coagulating bath. Also, the bath temperature may be slightly lower.

What I claim and desire to secure by United States Letters Patent is:

1. In a process for manufacturing artificial textile fibers from milk casein, following the spinning of an alkaline solution of such casein, the step of coagulating the spun filaments by treatment in an aqueous acid bath, containing a salt for promoting coagulation, selected from the group consisting of the sulphates of sodium and magnesium and zinc and ammonium; and containing a hardening and insolubilizing agent selected from the group consisting of aluminum sulphate and potash alum.

2. The process as in claim 1 and wherein the hardening and insolubilizing agent is aluminum sulphate.

3. In a process for manufacturing artificial textile fibers from milk casein, following the spinning of an alkaline solution of such casein, the step of coagulating the spun filaments by treatment in an aqueous acid bath, containing a salt for promoting coagulation, selected from the group consisting of the sulphates of sodium and magnesium and zinc and ammonium, and containing sodium chloride and aluminum sulphate to harden and insolubilize the coagulated filaments.

4. A process for making artificial textile fibers from an alkaline solution of casein which consist in spinning filaments of the soluble casein into an acid bath containing in each liter approximately 150 cubic centimeters of sulphuric acid of 66° Bé.; from 150 to 200 grams of aluminum sulphate, approximately 75 grams of sodium chloride and a minor quantity of magnesium sulphate.

ANTONIO FERRETTI